

## UNITED STATES PATENT OFFICE

HANS T. CLARKE AND CARL J. MALM, OF ROCHESTER, NEW YORK, ASSIGNORS TO EASTMAN KODAK COMPANY, OF ROCHESTER, NEW YORK, A CORPORATION OF NEW YORK

PROCESS OF ESTERIFYING CELLULOSIC MATERIALS WITH VAPORS OF LOWER FATTY ACIDS

No Drawing.

Application filed June 21, 1927. Serial No. 200,502.

This invention relates to processes of esterifying cellulosic materials with the vapors of the lower fatty acids containing more than one and less than eight carbon atoms. This application continues that subject matter which is common to it and our prior applications Serial No. 122,028, filed July 12th, 1926 for cellulose esters of fatty acids and processes of making the same, Serial No. 160,765, filed January 12th, 1927 for process of esterifying hydrated cellulose with lower fatty acids and Serial No. 186,170, filed April 23rd, 1927 for process of esterifying mercerized cellulose with lower fatty acids which are Letters Patent #1,668,944, 1,668,945 and 1,687,059 respectively.

One object of our invention is to provide an inexpensive and simple process of producing cellulose esters of the lower fatty acids without the aid of anhydrides or catalysts and under conditions which will not molecularly degrade the cellulose or the esters produced from it. Another object of the invention is to provide a process of making cellulose esters of the lower fatty acids in a plurality of stages, certain of the acid groups being combined into the ester during the first stage while the acids are in the vapor form and without the use of anhydrides and catalysts; and the remainder of the acid groups being combined in the ester by the subsequent treatment of the esters formed in the first stage, thus effecting an economy in expensive ingredients, such as the anhydrides of the fatty acids, and eliminating the manipulations incident to the treatments with the acids in liquid form. Still another object of the invention is to provide a process of esterifying cellulosic material by means of the vapors of the lower fatty acids at temperatures which produce rapid esterification and in the absence of oxygen or catalysts which would rapidly degrade cellulose and the cellulosic esters at such elevated temperatures. A further object is to provide a process of esterifying cellulosic material by means of the vapors of the lower fatty acids without subjecting said material to any esterifying or washing liquids during such esterification. Other objects will hereinafter appear.

We have found that the above objects may be attained by subjecting cellulosic material to vapors of one or more of the fatty acids containing more than one but less than eight carbon atoms at temperatures above 100° C. and below the temperature at which degradation of the product takes place,—say about 200° C. We have likewise found that the vapors of the acids should be substantially free from oxygen gas which causes very rapid deterioration of the cellulosic material and the cellulose esters at such high temperatures. It is also highly preferable that any catalyst, such as sulfuric acid, for example, be omitted during this vapor treatment, because of its well known deteriorating action on cellulosic materials at such temperatures.

We have likewise found that when at least 4% of acetyl groups are combined with the cellulose by our vapor treatment, the lower esters, thus produced, can be further acetylated and made chloroform-soluble, or acetone-soluble, by the customary methods, but with the amount of fatty acid anhydrid correspondingly diminished. Thus from the standpoint of the final product the preliminary vapor esterification effects a very great economy, because it is much cheaper than the anhydrid which it enables the manufacturer to dispense with. Moreover, it obtains this economy without degrading the material, as is evidenced by the flexibility of films made from the final product.

In our process we use the vapors of one or more of the fatty acids having more than one and less than eight carbon atoms, such as acetic, propionic, butyric, valeric, caproic, heptylic, etc. But the rate of esterification falls off rapidly with the higher members of this group of acids. While this can, to a considerable extent, be counteracted by working at as high a temperature as possible, nevertheless, we prefer to use the lower members of the group, such as acetic acid, propionic acid and butyric acid. Of these, acetic acid is commercially the most important at present, because of its lower cost.

For the cellulosic material we may use either plain cellulose, or mercerized cellulose, or hydrated cellulose obtained by reversion,

as in rayon manufacture. The esterification with acid vapors takes place most readily on the latter materials, and least readily on the plain cellulose, the ease of esterification of the mercerized cellulose varying with the manner in which the material has been dried. But while plain cellulose and mercerized cellulose are slower to vapor esterification, nevertheless the final cellulose acetates formed from them can, with more certainty, be relied upon to give flexible films. Consequently they are our preferred materials.

For the plain cellulose we may employ any of the types customarily used in the manufacture of esters, such, for instance, as cotton fibers, surgical cotton wool, tissue paper especially prepared from cotton, cotton linters, and even sulfite wood pulp of good quality (preferably bleached). During the treatment of such materials with the fatty acid vapors, the fibers or particles of cellulose do not materially swell or gelatinize, but retain substantially their original physical appearance.

Where the vapor esterification is employed with mercerized cellulose, the cellulosic materials, such as those mentioned in the immediately preceding paragraph, are first mercerized along customary lines. For one example, the mercerization may be conducted at room temperature by simply immersing the cellulose fibers in an aqueous solution of alkali, such as sodium hydroxide, of suitable concentration. With an 18% aqueous solution of sodium hydroxide we have obtained satisfactory results upon cotton fibers in twenty-four hours, but no harm was produced when a trial of such mercerization was continued for seventy-two hours. A mercerization in a 40% aqueous solution of sodium hydroxide is effective in twenty-four hours or less, without apparent degradation of the cellulose. After soaking in the alkaline solution at room temperature for the desired time, the solution is drained off, the mercerized cellulose fibers washed free from alkali with water, and then dried or dehydrated, preferably by displacing the water with alcohol followed by ether, or with benzol, and then evaporating off the latter, as set forth in our copending application Serial No. 186,169, filed April 23rd, 1927 for processes of making organic esters of cellulose.

The most useful range of temperatures lies between 100° C. and 200° C., provided that air or atmospheric oxygen be eliminated during the vapor treatment. But in the case of acetic acid especially, it is preferable to work above its boiling point, say above 117° C. It is a surprising fact that the pure vapors of acetic acid (free from air) will operate quickly at 150° C., without apparently degrading the cellulose or the lower cellulose acetate fibers which are produced. This is likewise

true of the other hereinabove mentioned acids below about 200° C.

The temperatures lying above the normal boiling points of the acids may be attained in one of two ways. In the first, the vapor may be generated in a closed system, in which a superatmospheric pressure is induced by introducing a suitable oxygen-free gas under pressure; the degree of excess pressure so obtained determines the temperature of the evolved vapor. In the second method, which is by far the more convenient, the vapor evolved on boiling at atmospheric pressure is superheated to the desired temperature before coming into contact with the cellulosic material. Loss of heat from the superheated vapor in the containing vessel is prevented by surrounding the latter with a steam or vapor jacket, electrically heated coil, or other suitable source of heat.

We shall now give several examples of our invention, but it will be understood that our invention is not restricted to the details thus set forth, except as indicated in the appended claims. The plain cellulose to be treated, say clean cotton fibers, is placed in a vessel constructed of material which is resistant to the vapors of the lower acids, such as aluminum, copper or glass-lined steel. The acid is heated in any suitable container and the vapors guided from it through a suitable superheater into the vessel containing the fibers to be treated. Care is taken to pass enough of the vapors into or through the cellulose-containing vessel to remove all the air before the temperature is raised to the working point. The temperature of the fibers is then raised to any desired point by suitable means, such as a steam or vapor jacket, or an electrically heated coil. We have found it advantageous to lead the vapors issuing from the vessel through a fractionating column, by which means any moisture present is allowed to escape from the system, the substantially anhydrous acid being returned to the distilling vessel, so that its vapor may again be passed through the cellulose-containing vessel, precaution always being taken to exclude air by the ample supply of fatty acid vapor. Working under these conditions at 140° C. we have obtained, for instance, an ester with well over 4% of acetyl content in six hours, and a full 6% of acetyl in as short a time as twenty hours.

In the above example mercerized fibers may be substituted in place of the plain, clean, cotton fibers. The acetylation then takes place still more rapidly and may be carried to a considerably higher limit. Ordinarily we prefer to carry the esterification of mercerized and dehydrated fibers above 8% of acetyl. When fibers of this degree of esterification are further acetylated in the usual way the economy in anhydrid is very great,

being between 20% and 40% in typical instances.

The highest speed of acetylation is obtained when the vapor treatment is carried out on fibers of rayon made by the viscose process, or the cuprammonium process or the denitrated nitro-cellulose process. These are examples of so-called "hydrated" cellulose. We do not like to use in our process any cellulose material which has been so degraded by hydrolysis or oxidation as to yield esters which form brittle films. Some care, therefore, is exercised in testing the rayon fibers which are suitable for producing good products by our processes. When suitable rayon fibers are treated, in the same way that the plain cellulose is treated in the hereinabove given example, the esterification by the vapors takes place relatively very rapidly and the percentage of acetyl in the fibers can be quickly brought above 8% so as to effect notable economies in subsequent complete acetylation.

While in the above examples we have mentioned 4% as the quantity of acetyl which allows a useful economy of anhydrid in subsequent operations, and have stated that we prefer to obtain 8% of acetyl when operating on mercerized fibers or rayon fibers, we, nevertheless, can obtain much higher acetyl values by merely prolonging the operation, and without serious molecular degradation of the materials. Working on mercerized cellulose, we have often obtained an acetyl content of above 20%.

Since our esterification by means of vapors leaves the fibers or particles of the various cellulose materials in substantially their original physical form, without causing them to swell or stick together, the handling of the materials is the simplest possible. They are merely put into the apparatus and then taken out at the end of the esterification, without any need of washing out an excess of acid, and thereby diluting and lowering the value of the latter. Nor is any drying step necessary.

The lower acetyl celluloses, or other lower esters of the fatty acids, obtained by means of the vapors, possess increased susceptibility to further esterification, the latter being effected in any suitable known way. Thus, for example, the subsequent acetylation to chloroform solubility can be carried out in a bath of acetic acid and acetic anhydrid containing zinc chloride or magnesium perchlorate trihydrate as the catalysts. In such a bath, of course, the percentage of anhydrid is cut down so as to be only 60% to 80% of that usually used.

Our vapor-esterified products are also useful in preparing mixed esters. Thus a cellulose acetate, prepared as hereinabove described and containing 8% of acetyl groups, may be further esterified in any of the baths

set forth in our copending application Serial No. 179,177, filed March 28th, 1927 for Process of Making Cellulose Esters of Organic Acids. Such baths comprise an organic acid (say from 10 to 25 parts by weight) such as propionic, n-butyric, iso-butyric, n-valeric, iso-valeric, n-caproic, n-heptylic, caprylic, pelargonic, capric, lauric, myristic, palmitic, stearic, crotonic, cyclohexanecarboxylic, benzoic, o-methoxy-benzoic, o-chloro-benzoic, acetyl salicylic, phenylacetic, hydrocinnamic, cinnamic, and 30 to 60 parts by weight of anhydride which impels esterification, such as chloroacetic anhydride, together with a catalyst, such as .05 parts by weight of magnesium perchlorate trihydrate. In this bath there are treated from 3 to 5 parts by weight of the cellulose material, the operation being conducted at 60° to 65° C. until a homogeneous dope is obtained, usually in from 3 to 24 hours. Or, again, a cellulose propionate containing 15% of propionyl (prepared by exposing mercerized cellulose to the action of propionic acid vapor at 160-165° C. for twenty hours) may be further esterified by means of acetic anhydrid in the presence of a suitable catalyst, when it yields an ester directly soluble in acetone.

Having thus described our invention, what we claim as new and desire to secure by Letters Patent is:

1. In the process of making a cellulose ester of a fatty acid, heating esterifiable cellulose material in the vapor of a fatty acid having more than one and less than eight carbon atoms at a temperature above 100° C. and below the temperature at which the product is degraded until the acetyl group in the ester thus produced reaches at least 4%, said vapor being the sole acetylating agent. 160

2. In the process of making a cellulose ester of a fatty acid, heating esterifiable cellulose material in the vapor of a fatty acid having more than one and less than eight carbon atoms at a temperature above 100° C. but less than 200° C. in the absence of oxygen gas and degrading catalysts until the acetyl group in the ester thus produced reaches at least 4%, said vapor being the sole acetylating agent. 110

3. In the process of making a cellulose ester of acetic acid, heating esterifiable cellulose material in the vapor of acetic acid at a temperature above 100° C. and below 200° C. in the absence of oxygen gas and degrading catalysts, until the acetyl group in the ester thus produced reaches at least 4%, said vapor being the sole acetylating agent. 115

4. In the process of making a cellulose ester of a fatty acid, heating esterifiable cellulose material in the superheated vapor of a fatty acid having more than one and less than eight carbon atoms at a temperature above 117° C. but below 200° C. in the absence of oxygen gas and degrading catalysts, until the acetyl group in the ester thus produced 130

reaches at least 4%, said vapor being the sole acylating agent.

5. In the process of making a cellulose ester of a fatty acid, heating mercerized cellulose in the vapor of a fatty acid having more than one and less than eight carbon atoms at a temperature above 100° C. but below the temperature at which the product is degraded, in the absence of oxygen gas, 10 until the acyl group in the ester thus produced reaches at least 8%, said vapor being the sole acylating agent.

6. In the process of making cellulose acetate, heating mercerized cellulose in acetic acid vapor at a temperature above 100° C. but below 200° C. in the absence of oxygen gas and degrading catalysts until the acetyl group in the ester thus produced reaches at least 8%, said vapor being the sole acetylating agent. 20

7. In the process of making a cellulose ester of a fatty acid, heating esterifiable cellulosic material in the vapor of a fatty acid having more than one and less than eight 25 carbon atoms at a temperature above 100° C. and below the temperature at which the product is degraded until the acyl group in the ester thus produced reaches at least 4%, said vapor being the sole acylating agent, and thereafter further esterifying the ester thus produced with additional acyl groups. 30

8. In the process of making a cellulose ester of a fatty acid, heating esterifiable cellulosic material in the vapor of a fatty acid having more than one and less than eight carbon atoms at a temperature above 100° C. but less than 200° C. in the absence of oxygen gas and degrading catalysts until the acyl group in the ester thus produced 35 reaches at least 4%, said vapor being the sole acylating agent, and thereafter further esterifying the ester thus produced with additional acyl groups by the aid of an anhydrid and a catalyst. 40

45 9. In the process of making a cellulose ester of acetic acid, heating esterifiable cellulosic material in the vapor of acetic acid at a temperature above 100° C. and below 200° C. in the absence of oxygen gas and degrading catalysts, until the acetyl group in the ester thus produced reaches at least 4%, said vapor being the sole acylating agent, and thereafter further esterifying the ester thus produced with additional acyl groups by the 50 aid of an anhydrid and a catalyst. 55

10. In the process of making a cellulose ester of a fatty acid, heating esterifiable cellulosic material in the superheated vapor of a fatty acid having more than one and less 60 than eight carbon atoms at a temperature above 117° C. but below 200° C. in the absence of oxygen gas and degrading catalysts, until the acyl group in the ester thus produced reaches at least 4%, said vapor being 65 the sole acylating agent, and thereafter fur-

ther esterifying the ester thus produced with additional acyl groups.

11. In the process of making a cellulose ester of a fatty acid, heating mercerized, cellulose in the vapor of a fatty acid having more than one and less than eight carbon atoms at a temperature above 100° C. but below the temperature at which the product is degraded in the absence of oxygen gas or degrading catalysts until the acyl group in the ester thus produced reaches at least 8%, and thereafter further esterifying the ester thus produced with additional acyl groups by the aid of an anhydrid and a catalyst. 70 75

12. In the process of making cellulose acetate, heating mercerized cellulose in acetic acid vapor at a temperature above 100° C. but below 200° C. in the absence of oxygen and degrading catalysts at superatmospheric pressure until the acetyl group in the ester 80 thus produced reaches at least 8%, and thereafter further esterifying the ester thus produced with a mixture containing acetic anhydrid and a catalyst. 85

Signed at Rochester, New York, this 16th 90 day of June, 1927.

HANS T. CLARKE.  
CARL J. MALM.

95

100

105

110

115

120

125

130

**CERTIFICATE OF CORRECTION.**

**Patent No. 1,823,350.**

**Granted September 15, 1931, to**

**HANS T. CLARKE ET AL.**

It is hereby certified that error appears in the printed specification of the above numbered patent requiring correction as follows: Page 3, line 38, for "cellulosis" read cellulosic; same page, line 103, claim 1, line 112, claim 2, and line 130, claim 4, for "acetyl" read acyl; same page, line 105, claim 1, line 114, claim 2, and page 4, line 2, claim 4, for "acetylating" read acylating; and that the said Letters Patent should be read with these corrections therein that the same may conform to the record of the case in the Patent Office.

Signed and sealed this 17th day of November, A. D. 1931.

(Seal)

**M. J. Moore,  
Acting Commissioner of Patents.**